

**1**

3,667,981

**UPGRADED CAST REFRACTORY PRODUCTS**  
Marc Roland Gilbert Esnoult, Le Pontet, and Michel Louis Ayme-Jouve, Sorgues, France, assignor to L'Electro-Refractaire, Paris, France  
No Drawing. Filed Dec. 23, 1969, Ser. No. 887,774  
Claims priority, application France, Dec. 27, 1968,  
181,380  
Int. Cl. E04g 23/02, 21/00  
U.S. Cl. 117—2 R 6 Claims

**ABSTRACT OF THE DISCLOSURE**

The invention relates to cast refractory products having dispersed shrinkage cavities or voids, these products being characterized in that said cavities or voids are filled with a suitable grout comprising powdered refractory materials.

Electrically fused, cast refractory products are well-known materials which are used, more especially in various industries, for the construction of certain parts of furnaces. Some of these products have the tendency, during their manufacture to give rise to a quite considerable shrinkage cavity or pipe, and it is customary to disperse the latter.

A typical example of these materials is the product sold commercially under the name of "Corhart 104" and described in United States patent specification No. 2,599,566, for which a typical composition is: 55-56% of MgO, 20% of Cr<sub>2</sub>O<sub>3</sub>, 12-13% of FeO, 7-8% of Al<sub>2</sub>O<sub>3</sub>, 2.5% of SiO<sub>2</sub> and 1.3% of CaO. This product is manufactured in the form of slabs, from which the commercial units are cut.

For these products, the dispersion of the shrinkage cavity is achieved by means of various well-known procedures, such as the introduction into the casting of the slabs of a certain amount of a small-grain substance made up of the material crushed up (a method described on page 247 of the English translation of the book by A. A. Litwakowski: "Fused Cast Refractories," 1961, or in French patent specification No. 738,117), or such as the introduction into the casting of the slabs of a product able to liberate gases (a method described in French patent specification No. 922,954), or in a combination of these methods.

This method of proceeding has a twofold result:

In respect of the economic effect, it makes it possible to cut from the slabs units suitable over almost their entire height, and to re-use defective units in the form of small grains; and

In respect of quality, it renders the quality homogeneous over almost the entire height of the slabs and, through the introduction of holes due to the distribution of the shrinkage cavity, to improve resistance to thermal fracturing in the material.

Holes formed in this way at the time of the dispersion of the shrinkage cavity are not without drawbacks, however; they spoil the appearance of the product, constitute relatively easier paths for the penetration of aggressive agents and, when the refractory is in contact with fluids in movement, give rise to turbulences and vortices which hasten the wearing down of the material.

The sole means hitherto known and employed for obviating these drawbacks was to bring compact blocks into being, but the improvement in the resistance to cor-

**2**

rosion obtained in this way was counter-balanced in respect of quality by a decreased resistance to thermal variations and, in respect of economic effect, by so great an increase in the costs of manufacture that the profitability of the product was no longer assured.

The present invention has for its object electrically fused, cast refractory products of improved appearance and quality, and the manufacturing cost of which is slightly less than that of products at present available.

According to the invention, the said refractory products are characterized in that the holes from the dispersed shrinkage cavity are filled in and made good by means of a suitable grout.

15 The filling-in and making good of the holes from the dispersed shrinkage cavity can be put into effect by various methods.

One of these methods consists in subjecting the block to be filled in (the sawn faces of which have been arranged horizontally) to horizontal vibrations or to vertical shocks, and to apply the grout with a trowel successively to the two sawn faces.

20 Another of the said methods consists in arranging the block requiring to be filled in in a chamber which can be de-pressurized, creating a vacuum in the said chamber, placing the chamber in communication with a source of grouting material while preventing the entry of air into the chamber so as to introduce the grout into the chamber and to fill the holes with grout, then interrupting the vacuum, removing the block, scraping it over and in recovering the remaining grout for the following operation. The block is then allowed to dry in the air or under any other appropriate conditions.

25 A further possible method consists in arranging the block to be filled in in a chamber which can be linked to a pressure source, introducing the grout into the chamber, and placing the chamber under pressure, after which the pressure is relieved, the block is removed and is scraped over, as in the previous instance. This method can moreover be usefully combined with the preceding one, 30 it being possible to effect the pressurization of the chamber after the introduction "in vacuo" of the grout. It is this latter method which constitutes the best way of filling in the refractory products which are the aim of the invention.

35 The conditions as regards vacuum and pressure are not critical. It is possible, for instance, to apply a vacuum of the order of 10 to 50 mm. of Hg by means of an impeller pump, and/or a pressure of the order of several atmospheres by making a connection to a source of compressed air.

40 The grout employed should naturally satisfy a number of conditions. In particular, it should not pour out excessively under the effect of the vibrations or shocks in question or of the suction of the liquid by the vacuum: it should be sufficiently fine to penetrate into the narrow orifices of the refractory product requiring treatment, but should not be too fine, so as to prevent too great a contraction upon drying; it should be thixotropic, so as not to run out of the external shrinkage holes after the treatment; it should not harden too rapidly in the presence of cold; it should harden in the presence of heat, so as not to collapse into powder at the commencement of the heating process when actually in use; it should be adequately resistant to corrosion. Various examples of grout 45 will be given hereinafter.

The filling-in and making good of the dispersed shrinkage holes is, in the case of a method for filling in and making good and for a given grout, all the better, the more extensive the communication between the holes is. Thus, though slabs of Corhart 104 prepared by the normal procedure may be treated in accordance with the invention so as to obtain slabs of improved quality, the present applicant has found that better results are achieved when the slabs are manufactured by a special method which leads to the formation of an open porosity in the final slabs. Such a method, for example, consists in dispersing the shrinkage cavity by the addition of small-grain material and by employing a fusion technique which brings about degasification of the bath of melted material of the kind described in French patent specification No. 1,208,577 and its addition, No. 75,893, 82,057, 82,310 and 84,153.

The refractory products according to the invention possess, in relation to the products whose dispersed shrinkage holes have not been filled in, an improved appearance, a density increased by approximately 5%, and a resistance to corrosion which is higher by about 15%. In another connection, the treatment covered by the invention makes it possible to decrease the effects of tur-

| Grout                                                                             | A  | B  | C     | D  |
|-----------------------------------------------------------------------------------|----|----|-------|----|
| Powder C 104, parts <sup>1</sup>                                                  | 88 | 88 | ----- | 25 |
| Alsing C 104, parts <sup>2</sup>                                                  | 7  | 7  | 94    | 25 |
| Slurries from sawing, parts                                                       |    |    |       | 50 |
| Commercial clay, parts                                                            | 1  | 1  | 1     | 1  |
| Sodium silicate in powder form ( $\text{SiO}_2/\text{Na}_2\text{O}=2$ ):<br>parts | 5  | 5  | 5     | 3  |

<sup>1</sup> The material concerned is the commercial product "Corhart 104," pulverized and passing through a sieve of 0.5 mm. mesh.

<sup>2</sup> The material concerned is the commercial product "Corhart 104," pulverized in an Alsing-Brand ball-mill and passing through a sieve of 0.1 mm. mesh.

To these compositions was added 15 to 20% approximately of water in order to obtain grouts of the appropriate consistency.

#### EXAMPLE 2

The grout A and B of Example 1 were employed in the carrying out of tests on the filling-in effect in respect of blocks of Corhart 104 specially manufactured to obtain a degassed product.

The filling-in method employed and the results obtained are shown in the table below. For each series of tests, the results have been classified according to increasing densities:

| Test No. | Method of filling-in employed used | Grout | Densities in g./cm. <sup>3</sup> |       | Average gain, g./cm. <sup>3</sup> |
|----------|------------------------------------|-------|----------------------------------|-------|-----------------------------------|
|          |                                    |       | Before                           | After |                                   |
| 1        | Horizontal vibrations <sup>1</sup> | A     | 3.10                             | 3.16  | 0.06                              |
| 2        |                                    |       | 3.18                             | 3.27  | 0.09                              |
| 3        |                                    |       | 3.24                             | 3.34  | 0.10                              |
| 4        |                                    |       | 2.97                             | 3.08  | 0.11                              |
| 5        |                                    |       | 3.06                             | 3.20  | 0.14                              |
| 6        |                                    |       | 3.15                             | 3.28  | 0.13                              |
| 7        | Vertical shocks <sup>1</sup>       | A     | 3.21                             | 3.28  | 0.07                              |
| 8        |                                    |       | 3.22                             | 3.28  | 0.06                              |
| 9        |                                    |       | 3.22                             | 3.34  | 0.12                              |
| 10       |                                    |       | 3.24                             | 3.36  | 0.12                              |
| 11       |                                    |       | 3.00                             | 3.18  | 0.18                              |
| 12       |                                    |       | 3.08                             | 3.19  | 0.11                              |
| 13       | Vertical shocks <sup>2</sup>       | B     | 3.12                             | 3.21  | 0.09                              |
| 14       |                                    |       | 3.16                             | 3.29  | 0.13                              |
| 15       |                                    |       | 3.19                             | 3.27  | 0.08                              |
| 16       |                                    |       | 3.22                             | 3.31  | 0.09                              |
| 17       |                                    |       | 3.22                             | 3.30  | 0.08                              |
| 18       |                                    |       | 2.96                             | 3.08  | 0.12                              |
| 19       | Vacuum (12-15 mm. of Hg)           | B     | 3.00                             | 3.18  | 0.18                              |
| 20       |                                    |       | 3.11                             | 3.34  | 0.23                              |
| 21       |                                    |       | 3.14                             | 3.25  | 0.11                              |
| 22       |                                    |       | 3.16                             | 3.32  | 0.16                              |
| 23       |                                    |       | 3.22                             | 3.34  | 0.12                              |

<sup>1</sup> The block to be treated was placed on a frame set vibrating by a pneumatic hammer

<sup>2</sup> The block to be treated was subjected to shocks of an amplitude equal to 3 cm. and at a frequency of 160 shocks per minute.

bulence, to increase resistance to thermal variations by acting on the distribution and the size of the porosity, and by diminishing the manufacturing cost through improving the yield and through re-utilizing the waste material and the slurries arising from the sawing, it being possible to incorporate the said waste and slurries in the composition of the grout.

The following examples, of a non-limitative character, are given with a view to illustrating how the invention operates. All the percentages or parts given are by weight unless otherwise stipulated.

#### EXAMPLE 1

The following table indicates the composition of the grouts employed for filling in the cavities or holes in refractory products with a base of chromium oxide and magnesium oxide.

Of the three filling-in methods employed for the treatment of these blocks, the method "in vacuo" yields the best results, with an average gain in density of 0.15 g./cm.<sup>3</sup>. The gain does not appear to depend especially on the initial density, but rather on the volume of the accessible holes or cavities, one large hole filling up better than several small ones.

In this series of tests, only the two first grouts A and B, with a large proportion of C 104 powder, were used, to avoid contraction in the large shrinkage holes. Grout B, which contains 1% of commercial clay, is slightly superior to grout A.

The blocks, duly filled in, are good enough to use.

#### EXAMPLE 3

Grouts A, B and C in Example 1 were used in carrying out tests on filling in blocks of Corhart 104, of stand-

ard manufacture, in order to improve their appearance and their quality. The method of filling employed and the results obtained are set out in the following table. For each series of tests, the results have been classified by increasing densities.

can be used, varying the relative proportion of C 104 powder, of Alsing C 104 and of slurries originating in the sawing of the Corhart 104 slabs. Likewise, it is possible to use grouts other than with a base of Corhart 104, for example with a magnesia base.

| Test No. | Method of filling-in employed                                   | Grout used | Densities in g./cm. <sup>3</sup> |       | Average gain, g./cm. <sup>3</sup> |
|----------|-----------------------------------------------------------------|------------|----------------------------------|-------|-----------------------------------|
|          |                                                                 |            | Before                           | After |                                   |
| 24       |                                                                 | A          | 2.99                             | 3.04  | 0.05                              |
| 25       |                                                                 | A          | 3.02                             | 3.08  | 0.06                              |
| 26       |                                                                 | A          | 3.13                             | 3.18  | 0.05                              |
| 27       | Vertical shocks <sup>1</sup>                                    | B          | 3.15                             | 3.21  | 0.06                              |
| 28       |                                                                 | B          | 3.18                             | 3.25  | 0.07                              |
| 29       |                                                                 | B          | 3.27                             | 3.33  | 0.06                              |
| 30       |                                                                 | B          | 3.30                             | 3.36  | 0.06                              |
| 31       |                                                                 | B          | 3.21                             | 3.31  | 0.10                              |
| 32       |                                                                 | B          | 3.33                             | 3.39  | 0.06                              |
| 33       | Vacuum (12-15 mm. of Hg)                                        | C          | 3.27                             | 3.37  | 0.10                              |
| 34       |                                                                 | C          | 3.28                             | 3.41  | 0.13                              |
| 35       |                                                                 | C          | 3.35                             | 3.47  | 0.12                              |
| 36       | Pressure, (4.5 kg./cm. <sup>2</sup> )                           | C          | 3.22                             | 3.32  | 0.10                              |
| 37       |                                                                 | C          | 3.23                             | 3.30  | 0.07                              |
| 38       |                                                                 | C          | 3.18                             | 3.35  | 0.17                              |
| 39       |                                                                 | C          | 3.22                             | 3.33  | 0.11                              |
| 40       | Vacuum (15 mm. of Hg) plus pressure (4.5 kg./cm. <sup>2</sup> ) | C          | 3.23                             | 3.37  | 0.14                              |
| 41       |                                                                 | C          | 3.24                             | 3.38  | 0.14                              |
| 42       |                                                                 | C          | 3.24                             | 3.38  | 0.14                              |

<sup>1</sup> The block to be treated was subjected to shocks with an amplitude equal to 3 cm. and with a frequency of 160 shocks per minute.

Comparison of the tables in Examples 2 and 3 clearly shows that, for one and the same grout and the same method of filling in, the Corhart 104 of special manufacture leads to better filling in.

In another connection, the table in Example 3 shows that the best method of filling in is carried out "in vacuo," followed by pressurization. Grout C with a finer grain-size is superior to grout B from the point of view of penetration, as the results of tests 31 to 35 show. Grout C however, has the drawback of being more awkward and of suffering from greater contraction upon being dried.

#### EXAMPLE 4

In place of grout C, which has certain drawbacks (a high cost of manufacture and considerable contraction upon being dried), grout D can be employed. This grout was tried on blocks of special manufacture and, as in the other tests, the results have been classified by increasing densities:

| Test No. | Method of filling-in employed                                   | Grout used | Densities in g./cm. <sup>3</sup> |       | Average gain, g./cm. <sup>3</sup> |
|----------|-----------------------------------------------------------------|------------|----------------------------------|-------|-----------------------------------|
|          |                                                                 |            | Before                           | After |                                   |
| 43       |                                                                 |            | 3.22                             | 3.35  | 0.13                              |
| 44       |                                                                 |            | 3.23                             | 3.35  | 0.12                              |
| 45       | Vacuum (15 mm. of Hg) plus pressure (4.5 kg./cm. <sup>2</sup> ) | D          | 3.24                             | 3.38  | 0.14                              |
| 46       |                                                                 |            | 3.24                             | 3.39  | 0.15                              |
| 47       |                                                                 |            | 3.26                             | 3.38  | 0.12                              |
| 48       |                                                                 |            | 3.26                             | 3.43  | 0.17                              |

Grout D leads to results which are slightly inferior to those with grout C (the average gain is the same, but the results given by grout C refer to normal blocks, whereas those of grout D relate to special blocks). Nevertheless, grout D constitutes the best comprise from the point of view of quality/cost of manufacture.

The aforementioned examples show that the size of the holes and the porosity of the blocks has a preponderating influence on the gain in density achieved.

Naturally, other grouts can be used in place of the particular grouts indicated. In particular, intermediate grouts

| Attacking agent                                            | Product                                               | Corrosion indices |
|------------------------------------------------------------|-------------------------------------------------------|-------------------|
| Iron scale at 1,680° C. for 3 hours duration.              | Untreated C 104 ---<br>C 104 treated with<br>grout A. | 64<br>77          |
| Basic slag <sup>1</sup> at 1,680° C. for 3 hours duration. | Untreated C 104 ---<br>C 104 treated with<br>grout A. | 64<br>73          |

<sup>1</sup> FeO, 30%; CaO, 50% and SiO<sub>2</sub>, 20%.

It is self-evident that the methods described for carrying the invention into effect are only examples and that it would be possible to modify them, more especially by substituting technically equivalent means, without however thereby going beyond the scope of the invention.

65 We claim:

1. Cast refractory products of any known oxide-based composition having dispersed shrinkage cavities therein, characterized in that said cavities are filled with a heat-hardenable, thixotropic grout comprising, as main solid components, at least one powdered refractory oxide selected among the main oxides contained in the composition of said cast refractory products.

2. Cast refractory products of any known oxide-based composition having dispersed shrinkage cavities therein, characterized in that said cavities are filled with a heat-

hardenable, thixotropic grout comprising, as main solid components, powdered refractory materials having a composition similar to that of the said refractory product.

3. Cast refractory products comprising, by weight, about 55-56% MgO, about 20% Cr<sub>2</sub>O<sub>3</sub>, about 12-13% FeO, about 7-8% Al<sub>2</sub>O<sub>3</sub>, about 2.5% SiO<sub>2</sub> and about 1.3% CaO, and having dispersed shrinkage cavities therein, characterized in that said cavities are filled with a heat hardenable, thixotropic grout comprising, as main solid components, powdered refractory materials having a composition similar to that of the cast refractory products.

4. Process for upgrading cast refractory products of any known oxide-based composition having dispersed shrinkage cavities therein, characterized by filling said cavities with a heat-hardenable, thixotropic grout comprising, as main solid components, at least one powdered refractory oxide selected among the main oxides contained in the composition of said cast refractory products.

5. Process for upgrading cast refractory products of any known oxide-based composition having dispersed shrinkage cavities therein, characterized by filling said cavities with a heat-hardenable, thixotropic grout comprising, as main solid components, powdered refractory materials having a composition similar to that of the cast refractory product.

6. Process for upgrading cast refractory products comprising, by weight, about 55-56% MgO, about 20% Cr<sub>2</sub>O<sub>3</sub>, about 12-13% FeO, about 7-8% Al<sub>2</sub>O<sub>3</sub>, about 2.5% SiO<sub>2</sub> and about 1.3% CaO, and having dispersed shrinkage cavities therein, characterized by filling said cavities with a heat-hardenable, thixotropic grout comprising, as main solid components, powdered refractory materials having a composition similar to that of the cast refractory products.

#### References Cited

##### UNITED STATES PATENTS

|           |         |               |           |
|-----------|---------|---------------|-----------|
| 707,670   | 8/1902  | Zuckschwerdt  | 117-123 A |
| 2,968,083 | 1/1962  | Lentz et al.  | 117-2 R   |
| 3,141,790 | 7/1964  | Davies et al. | 117-123 A |
| 2,534,328 | 12/1950 | Whitman       | 117-169 R |
| 2,187,324 | 1/1940  | Many          | 117-2 R   |

ALFRED L. LEAVITT, Primary Examiner

M. F. ESPOSITO, Assistant Examiner

U.S. Cl. X.R.

117-123 A, 169 R; 52-744